

## UNITED STATES PATENT OFFICE

2,579,436

## PROCESS OF INHIBITING THE DEGRADATION OF PHOTOGRAPHIC COLOR IMAGES

E. Scudder Mackey, Binghamton, N. Y., assignor to General Aniline &amp; Film Corporation, New York, N. Y., a corporation of Delaware

No Drawing. Application April 12, 1950,  
Serial No. 155,558

6 Claims. (Cl. 95—88)

1

This invention relates to the treatment of color photographs and especially to final rinse baths for inhibiting the color decomposition of azo, azine, azomethine, indophenol, and quinonimine dyes present in color photographic emulsions.

Despite the ordinary precautions taken in storing color photographs and prints, the color balance is often altered by heat, extreme humidity conditions and residual processing chemicals. This lack of color stability is very undesirable as valuable color records are rendered useless. The deterioration occurs as a yellowing or browning of the color photograph if storage is in a heated atmosphere. Another photographic dye fading condition often results in the loss of yellow or other color dyes. This condition is caused by high temperature and high humidity. For instance, the storing of colored photographs in an attic or even in a wallet often produces this undesirable color deterioration. It has been determined that color prints, particularly the white, will stain a brown because of oxidation of the color developing agent retained in the subbing layer and in dye clumps. Prints processed without the color development step do not exhibit this stain. These undesirable effects are frequently observed in the color photographs containing azomethine dyes. The changes naturally restrict the storage conditions while methods of increasing the resistance of these dyes to extreme humidity and residual chemical fading are of great commercial importance.

An object of my invention is to provide a novel method of treating colored photographs so that extreme humidity conditions do not destroy the original coloration.

Another object of my invention is to obtain color photographs whose colors are stable to heat as well as to the deteriorating effect of residual color developing chemicals.

Other objects and advantages will become apparent as the description proceeds.

I have found that the above objects are accomplished by employing as a final rinse bath an aqueous solution containing a stain inhibiting amount of a water-soluble hydantoin compound characterized by the following general formulae:



2



wherein R represents either hydrogen or methylol ( $\text{CH}_2\text{OH}$ ) group,  $\text{R}_1$  represents a lower alkyl group, e. g., methyl, ethyl, propyl, isopropyl, etc.,  $\text{R}_2$  represents a lower alkyl group of the same values as  $\text{R}_1$  or lower alkoxyalkyl group, e. g., methoxymethyl, ethoxyethyl, propoxypropyl, etc.,  $\text{R}_3$  represents either hydrogen or lower alkyl group of the same value as in  $\text{R}_2$ , and Z represents the divalent methylene radicals necessary to complete a 5- or 6-membered cycloaliphatic group, such as cyclopentyl or cyclohexyl and the water-soluble formaldehyde addition products of said hydantoin compound.

20 The following are examples of suitable hydantoins which may be employed for the purpose herein set forth:



60

(7)



5-methyl-5-ethoxyethylhydantoin.

(8)



or



1(or 3)-methol-5,5-dimethylhydantoin

The water-soluble resinous addition products of formaldehyde and hydantoins are readily prepared according to the process described in United States Patent 2,155,863, which discloses examples of such compounds contemplated for use herein.

This finding makes it possible to render color developed multicolor photographic material practically immune to the deteriorative effects of storage or aging while unaffected the original color balance. The extreme humidity fading characteristics of developing multicolor photographic materials containing azo, azine, azomethine, indophenol, and quinonimine dyes are substantially improved by subjecting the processed color photographs or transparencies to treatment with aqueous solutions of said hydantoins. When such solutions are employed as final rinse baths, i. e., after the complete processing of multicolor material, they will inhibit the color loss of color photographs which have been exposed to extreme humidity conditions, accelerated aging, or acid vapors when effecting the original color balance.

The concentration of the hydantoin compound may be varied from as little as .5% to as much as 20%. Amounts higher than the latter give little improvement. Concentrations ranging between 2 and 5% yield satisfactory results. The time of rinsing may also vary between 1 to 10 minutes. However, best results with a 3% solution are obtained when the bathing of the processed film is from 3 to 5 minutes. In developing solutions, the hydantoin compounds may be employed in acid, neutral, or alkaline media. Solutions having a pH of about 8 are, however, preferred.

The photographic multicolor materials, which may be processed with the anti-stain bath of the present invention are color reversible film, color negative film, color reversible white printing material coated on an opaque base, and color positive printing material coated on paper, irrespective of whether the dyestuff images are produced with color formers present in the emulsion, or by a selective second exposure followed by development with developing solutions containing color formers and color developing agents.

The color reversible film consists of an integral tri-pack emulsion coated on the usual clear cellulose acetate or nitrate film base. Each of the emulsions is sensitized to one of the primary colors of light, namely, blue, green, and red. The

top layer is blue sensitive. A filter layer, yellow in color and blue absorbing, lies under the top layer. Below this filter layer, lies a green sensitive emulsion layer, and below this is a red sensitive emulsion layer. Each of the three silver halide emulsion layers contains dye forming compounds which unite during the development of a silver image in an aromatic amine developing agent to form a dye with the oxidation product of the developing agent, or may be free from color formers in which case the film is processed with the color formers in the color developers by the selective second exposure and color development method as described in United States Patents 1,897,866, 1,900,870, 1,928,709, and 1,980,941.

As silver is formed during development, it must be removed after color development by treatment in a bleach, followed by treatment in a bath of sodium thiosulfate, according to usual practice.

20 A yellow dye is formed in the blue sensitive emulsion; a magenta dye is formed in the green sensitive emulsion; and a cyan dye is formed in the red sensitive emulsion. Combinations of these three printing primaries will produce all of the other colors in the finished film or print.

The color negative film is made up in the same manner as the color reversible film with the exception that it may contain a layer of clear gelatin between the red sensitive layer and the

30 green sensitive layer. The color reversible white opaque material is prepared in the same manner as color reversible film and the color negative film with the exception that the base consists of an opaque white film. The color paper is also constructed in the same manner as the color reversible film and the color negative film, with the exception that the emulsion is coated on a baryta coated paper base. Suitable methods for the preparation of photographic multilayer materials 35 have been described in the literature relating to color photography and are, therefore, not described here.

40 Multicolor photographic materials which are color developed by azine developers, i. e., aromatic triamines, to yield azine (phenazonium) dye images are described in United States Patent 2,486,440.

45 Multicolor photographic materials in which the final dye images are azo dye images are prepared according to the procedural steps disclosed in United States Patents 1,985,344 and 2,020,775.

50 The following examples describe in detail the methods for accomplishing the above objects, but it is to be understood that they are inserted 55 merely for the purpose of illustration and are not to be construed as limiting the scope of the invention.

#### Example I

60 A 2 1/4" x 2 1/4" color transparency was printed by projection on two 3" x 5" sheets of color reversible white opaque film having gelatin layers on both sides of the film base. The two exposed 65 color reversible white opaque film sheets were first developed for 12 minutes at 68° F. in a developer of the following composition:

|                                 |        |    |
|---------------------------------|--------|----|
| p-Monomethylaminophenol sulfate | grams  | 3  |
| Sodium sulfite                  | do     | 50 |
| Hydroquinone                    | do     | 6  |
| Sodium carbonate (monohydrate)  | do     | 40 |
| Sodium thiocyanate              | do     | 2  |
| Potassium bromide               | do     | 2  |
| Water to make                   | liters | 1  |

## 5

The developed film was shortstopped for 3 minutes at 68° F. in a 5% aqueous solution of sodium bisulphite.

The film was washed for 2 minutes in running water at 68° F. and re-exposed to white light.

The re-exposed film was color developed for 15 minutes at 68° F. in a developer of the following composition:

|                                         |        |    |
|-----------------------------------------|--------|----|
| p-Aminodiethylaniline monohydrachloride | grams  | 4  |
| Sodium sulfite                          | do     | 20 |
| Hydroxylamine hydrochloride             | do     | 2  |
| Sodium carbonate                        | do     | 80 |
| Potassium bromide                       | do     | 1  |
| Water to make                           | liters | 1  |

The color developed film was rinsed for 4 minutes in running water at 68° F. and hardened for 5 minutes in a 3% aqueous solution of potassium chrome alum.

The hardened film was washed for 5 minutes in running water at 68° F. The washed material was then treated with a bleach bath of the following composition:

|                                     |                   |     |
|-------------------------------------|-------------------|-----|
| Dipotassium monosodium ferricyanide | grams             | 100 |
| Potassium bromide                   | do                | 15  |
| Disodium phosphate                  | do                | 40  |
| Sodium bisulfite                    | do                | 25  |
| Formalin (40%)                      | cubic centimeters | 20  |
| Water to make                       | liters            | 1   |

The bleached film was washed for 5 minutes at 68° F. and then fixed for 5 minutes in a solution of the following composition:

|               |        |     |
|---------------|--------|-----|
| Hypo          | grams  | 200 |
| Borax         | do     | 10  |
| Water to make | liters | 1   |

After fixing, the material was washed for 10 minutes in running water at 68° F.

After the final washing, one print was allowed to dry while the other was rinsed for 3 minutes in an alkaline aqueous solution consisting of 98 parts by weight of water and 2 parts by weight of 5,5-dimethylhydantoin-formaldehyde resin prepared as described in Example I of United States Patent 2,155,863, and a sufficient amount of sodium carbonate (monohydrate) to adjust the pH to 7.8. The treated print was then allowed to dry.

Both prints, i. e., the treated and untreated, were exposed to high humidity oven conditions for 5 hours. During this time, the relative humidity in the oven ranged progressively from 56 to 100% at a temperature ranging from 40 to 60° C. The prints were removed from the oven and allowed to reach room temperature. It was observed that a very slight yellowing appeared on the treated color print. The color balance of the untreated color print, however, was completely ruined by a yellow stain appearing overall while at the same time the densities of the original yellow image were lowered. It was also noted that the back of the treated print was free of the yellow-brown stain which had appeared on the untreated sample.

## Example II

Example I was repeated with the exception that the high humidity oven test was replaced by a storage test. Both prints, i. e., the treated and untreated, were stored in an ordinary filing cabinet for over 8 months. Upon inspection, it was noted that the untreated print had stained a

## 6

brown-yellow in the white areas. This brown-yellow stain was very noticeable on the back of the untreated print. The images on the treated print had not yellowed nor did the back of the print show the yellow-brown stain which was so noticeable on the untreated print.

## Example III

Example I was repeated with the exception that 10 parts by weight of 5,5'-dimethylhydantoin-formaldehyde resin was replaced by the same weight of 1-methylol-5,5-dimethylhydantoin. The untreated print, after being subjected to the high humidity oven test was completely ruined whereas the treated print showed no noticeable discoloration.

## Example IV

Example I was repeated with the exception that the colored material employed was a color paper 20 and the final rinse bath was a 2% solution of dimethylhydantoin instead of a 2% solution of 5,5-dimethylhydantoin-formaldehyde resin. The color print which was allowed to dry without treatment showed yellow stain appearing overall after 25 being subjected to the high humidity oven test whereas the treated print was free of a yellow stain.

## Example V

Example I was repeated with the exception that 30 the final rinse bath was a slightly alkaline 3% solution of 5-methylhydantoin instead of a 2% solution of 5,5-dimethylhydantoin-formaldehyde resin. The untreated film, after being subjected to the high humidity oven test, showed an overall 35 yellow stain and as a result the color balance was completely ruined, whereas the treated film showed no staining whatsoever.

The above specific examples are to be regarded 40 as being merely illustrative of the invention and not in any sense restrictive. It will be obvious to those skilled in the art that many modifications, such as substituting equivalent materials and varying the proportions of the materials used, may be made. The scope of the invention is to be 45 limited solely by the appended claims.

I claim:

1. In the process of producing color photographic images in a multicolor photographic emulsion by exposing the emulsion, color developing, bleaching, fixing and washing the same, the improvement which comprises preventing the formation of stain after the washing operation by rinsing the said colored picture with an aqueous solution containing, in an anti-staining amount, a hydantoin compound selected from the class consisting of those corresponding to the following formulae:



wherein R represents a member selected from the class consisting of hydrogen and methylol group, R<sub>1</sub> represents a lower alkyl group, R<sub>2</sub> is a group selected from the class consisting of lower alkyl and lower alkoxyalkyl groups, R<sub>3</sub> represents a member selected from the class consisting of hydrogen and lower alkyl group, Z represents the methylene radicals necessary to complete a member selected from the class consisting of five-membered and six-membered cycloaliphatic groups, and the water-soluble formaldehyde addition products of said hydantoin compound.

2. The process according to claim 1 wherein the hydantoin compound is 5-ethylhydantoin.

3. The process according to claim 1 wherein the hydantoin compound is 5,5-dimethylhydantoin.

4. The process according to claim 1 wherein the hydantoin compound is 5,5-methylhydantoin.

5. The process according to claim 1 wherein the hydantoin compound is 1-methylol-5,5-dimethylhydantoin.

6. The process according to claim 1 wherein the hydantoin compound is 5,5-dimethylhydantoin-formaldehyde resin.

E. SCUDDER MACKEY.

No references cited.